

1,357,782.

H. KOPPERS,  
CRUCIBLE TREATMENT OF METALS,  
APPLICATION FILED SEPT. 3, 1920.

Patented Nov. 2, 1920.

FIG. 1.



FIG. 2.



Witness:

John H. Johnson

Inventor:

Heinrich Koppers,  
By: Munsey, Clark & Carpenter, U.S.A.

# UNITED STATES PATENT OFFICE.

HEINRICH KOPPERS, OF ESSEN-ON-THE-RUHR, GERMANY, ASSIGNOR TO THE  
KOPPERS DEVELOPMENT CORPORATION, A CORPORATION OF PENNSYLVANIA.

## CRUCIBLE TREATMENT OF METALS.

1,357,782.

Specification of Letters Patent.

Patented Nov. 2, 1920.

Application filed September 3, 1920. Serial No. 408,082.

*To all whom it may concern:*

Be it known that I, HEINRICH KOPPERS, (assignor to THE KOPPERS DEVELOPMENT CORPORATION, of Pennsylvania,) a citizen of 5 Germany, residing in Essen-on-the-Ruhr, Germany, have invented a new and useful Improvement in Crucible Treatments of Metals, of which the following is a specification.

10 This invention relates to the treatment of metals, such as iron and its alloys, in crucibles and has for one of its objects to effect efficient refining, including desulfurization of the metal and to obtain a high grade 15 product containing a minimum proportion of sulfur.

The presence of sulfur, especially in iron and its alloys, greatly impairs the quality of the metal, when occurring in other than 20 extremely small proportions. When present in iron, sulfur makes the iron much more liable to rust; in fact, the tendency of iron to deteriorate when exposed to atmospheric conditions is augmented by the presence of sulfur which constitutes an important factor in promoting such deterioration. In the case of steel, the presence of sulfur not only makes the steel liable to 25 rust, but imparts a brittle quality to the steel making it difficult to shape and impairing its strength. Consequently, it is of great importance in the metallurgical industry to restrict the quantity of sulfur in such metals as iron and steel to mere traces. 30 This invention provides a novel and improved treatment of the metal in a crucible furnace, by which treatment the sulfur content in the product of the crucible is limited to mere traces which do not appreciably impair the quality of the metal.

40 The invention has for other objects such other improvements or advantages in operation and such other advantageous results as may be found to obtain in the improved processes and apparatus hereinafter described as illustrative examples.

45 In the accompanying drawings, forming a part of this specification, and showing, for purposes of exemplification, a preferred 50 manner in which the invention may be embodied and practised, but without limiting the claimed invention specifically to such illustrative instance or instances:

55 Figure 1 is a vertical section through a diagrammatic representation of a crucible

or refining vessel for practising the improvements of the present invention; and

Fig. 2 is a horizontal section of the same on the line 2—2 of Fig. 1.

The same characters of reference indicate 60 the same parts throughout the several views.

Referring to said Figs. 1 and 2, the reference numeral 11 represents a crucible constructed of refractory material and having a lower chamber 12. Above the lower 65 chamber 12 and separating it from an upper chamber 13 is a horizontal foraminous partition 14 formed of refractory material, such as the clay or silica refractories ordinarily employed in this art. Through the 70 holes in the partition 14, superheated molten iron charged into the chamber 13 passes in small drops, or in the form of a spray, and is uniformly distributed throughout the area of a mass of slag which is charged 75 into the crucible in a superheated molten state. The slag mass, indicated at 15, stratifies on top of the molten metal stratum 16 in the bottom of the lower chamber 12. The level of the slag stratum 15 is maintained 80 just below the partition 14 by a slag overflow duct 17 which fixes the slag level. Immersed in the slag are pieces of incandescent carbon, such as coke, which may be introduced into the slag through an inlet 18 in 85 the side of the crucible. The inlet 18 is kept normally closed by means of a plug of any suitable character.

In addition to its neutralizing action on 90 the acidity of the ash contained in the coke, the lime stone slag stratum has an affinity for sulfur and such property of the slag to absorb sulfur is augmented by contact of incandescent carbon which, because of the level maintained by the overflow pipe 17 and 95 the partition 14, dips into the slag stratum. The incandescent carbon dipping into the superheated molten slag stratum constitutes a reduction medium that liberates elements having a deoxidizing effect on the iron. The 100 molten metal discharged in small drops, or in the form of a spray from the bottom of the partition 14, flows downwardly through and is subjected to the prolonged action of the solid incandescent carbon and slag, and 105 during such flow through the slag stratum a reaction is effected between the basic compounds present in the slag and the sulfur contained in the metallic iron, causing sulfur to be absorbed from the iron and to be re- 110

tained by the slag, with which the sulfur combines to form principally the compound, calcium sulfid. The absorption of sulfur by the slag may be illustrated, for example, by 5 the following two equations:



From these two equations, it will be observed 10 that the incandescent carbon induces the reaction resulting in the formation of calcium sulfid and pure iron. The calcium sulfid is soluble in and will be retained by the slag. The importance of the presence of incandescent carbon is illustrated by the first formula given above inasmuch as the action of the carbon is first to reduce the calcium oxid to metallic calcium, thereby augmenting the affinity of the slag stratum for absorption of 15 sulfur from the metal which passes through the slag.

In accordance with the invention, the above described factors which augment desulfurization of the iron are maintained continuously in their condition of maximum effect as regards desulfurization, during operation of the crucible. In order to effect this result and to secure a maximum desulfurizing effect promoted by the action of the 20 slag and immersed carbon, the invention provides for the maintenance of a continuous mass of slag in the lower chamber of the crucible. By the invention the iron obtained contains only small traces of sulfur. The 25 partition 14 keeps the incandescent carbon continuously immersed in the slag to maintain the slag at all times in its condition of maximum affinity for absorption of sulfur. The molten metal is discharged from the 30 bottom of the hearth through an overflow duct 19 which leads first upwardly and thence downwardly to a receiving vessel 20 for the molten metal. The fixed slag overflow duct 17 will determine the height of 35 the slag level in the crucible, whereas the fixed location of the crest 21 of the metal overflow duct 19 will determine the height of molten metal in the crucible, thereby maintaining constant levels both of slag and 40 molten metal in the crucible. In practice, the relation of these respective heights may be expressed as follows: the height of the crest of the overflow pipe above the junction with the hearth of the furnace equals the 45 height of the molten metal in the furnace above the junction point of the overflow pipe plus two-sevenths of the height of the slag stratum in the lower chamber of the furnace, assuming that the specific gravity 50 of the slag be two and that of the iron be seven.

The invention as hereinabove set forth may be practised in various ways without departing from the scope of the claims hereinafter made.

I claim:

1. A crucible for the treatment of metals, such as iron or its alloys, comprising: a vessel; a foraminous partition dividing said vessel into upper and lower compartments, to cause molten metal charged in the upper compartment to flow through the lower compartment in the form of a spray; and means for maintaining the slag and molten metal in the lower compartment respectively at 70 constant levels; substantially as specified.

2. A crucible for the treatment of metals, such as iron or its alloys, comprising: a vessel; a foraminous partition dividing said vessel into upper and lower compartments, 80 to cause molten metal charged in the upper compartment to flow through the lower compartment in the form of a spray; and constant-outflow means for permitting separate discharge of the slag and metal from said 85 lower compartment; substantially as specified.

3. A crucible for the treatment of metals, such as iron or its alloys, comprising: a vessel; a foraminous partition dividing said 90 vessel into upper and lower compartments, to cause molten metal charged in the upper compartment to flow through the lower compartment in the form of a spray; and overflow means communicating with said lower 95 compartment.

4. A crucible for the treatment of metals, such as iron or its alloys, comprising: a vessel; a foraminous partition dividing said vessel into upper and lower compartments, 100 the upper compartment receiving the molten metal and the lower compartment having an inlet for coke, said partition causing distribution of the molten metal in the form of a spray through the slag stratum in the 105 lower compartment and also maintaining the coke submerged in the slag stratum; and means for maintaining the slag and molten metal in the lower compartment respectively at constant levels; substantially as specified. 110

5. In the treatment of metals, such as iron or its alloys, a vessel in which molten slag stratifies on top of the mass of molten metal, means for converting the molten metal, introduced into said vessel, into the form of 115 a spray, for permitting the small particles of metal to pass and be distributed through the slag stratum, and separate outflow means for discharging the metal and slag from said vessel; substantially as specified.

6. The improved process of refining metals, such as iron and its alloys, which consists in converting the molten metal into the form of a spray, and passing the spray of molten metal through a molten slag stratum 125 having an affinity for sulfur, substantially as specified.

7. The improved process of refining metals, such as iron and its alloys, which consists in converting the molten metal into 130

the form of a spray, and uniformly distributing the spray of molten metal through a molten slag stratum having an affinity for sulfur, substantially as specified.

5 8. The improved process of refining metals, such as iron and its alloys, which consists in converting the molten metal into the form of a spray, and passing the spray of molten metal through a slag stratum in the 10 presence of incandescent carbon, substantially as specified.

9. The improved process of refining metals, such as iron and its alloys, which consists in converting the molten metal into the 15 form of a spray, and passing the spray of molten metal through a slag stratum in which incandescent carbon is submerged, substantially as specified.

10. The improved process of refining metals, such as iron and its alloys, which consists in converting the molten metal into the 20 form of a spray, and passing the spray of molten metal through a bath of basic slag in which incandescent carbon is submerged, substantially as specified.

25 11. An apparatus for desulfurizing metals, such as iron and its alloys, comprising: a vessel for containing the metal and slag, overflow means for the metal and slag for maintaining constant levels respectively of 30 the metal and superposed slag, and means for maintaining carbon submerged in the slag and for distributing the molten metal through the slag in the form of a spray.

HEINRICH KOPPERS.